

Oct. 7, 1941.

P. A. E. ARMSTRONG ET AL

2,258,563

PROCESS FOR MAKING STAINLESS CLAD PIERCED TUBES

Filed March 11, 1940



INVENTORS  
Percy A. E. Armstrong  
Tecumseh Sherman Fitch  
BY Alan M. Main  
ATTORNEY

## UNITED STATES PATENT OFFICE

2,258,563

PROCESS FOR MAKING STAINLESS CLAD  
PIERCED TUBESPercy A. E. Armstrong, Westport, Conn., and  
Tecumseh Sherman Fitch, Washington, Pa.;  
said Fitch assignor to said Armstrong

Application March 11, 1940, Serial No. 323,258

4 Claims. (Cl. 29—188)

This application relates to a method of producing composite steel tubes in which the lining is of a high melting point corrosion resistant metal such as nickel or a chromium alloy and the outer shell is a mild or low carbon steel. The composite tubes made in accordance with the process covered by this application are claimed in our divisional application Ser. No. 388,634, filed April 15, 1941.

The need for tubes of this kind has been recognized and heretofore attempts to make them have been undertaken in accordance with which an annular steel billet was prepared with a cylindrical core of corrosion resistant metal and this composite product was intended to be pierced on a standard Mannesmann mill. The difficulty with such a process is that the strain exerted in the piercing operation is sufficient to tear apart any bond that may exist between the cylindrical core and the outer annular shell.

In accordance with our invention, we start with a core of corrosion resistant metal which instead of being cylindrical is square in cross section, or has a cross section which is of an angular nature such as a hexagon or octagon. This is enclosed (either by casting or, preferably, in the manner later illustrated) in an outer shell of a steel which ordinarily will be corrodible and relatively ductile such as a low carbon or low alloy steel, which is also preferably square or at least is formed with oppositely disposed flat sides which permit the composite body to be rolled between flat faced rolls. This flat rolling effects a weld between the core and the outer cover. In order to assure that such a weld will be accomplished, the corrosion resistant metal (or even better, both the corrosion resistant metal and the faces of the corrodible metal that are to be welded with it) should first be electroplated with iron under conditions which will prevent the formation of a layer of intervening oxide as set forth in Armstrong Patent No. 1,997,538, dated April 9, 1935.

By hot rolling the original assembly or billet on its flat sides, an excellent bond or weld can be obtained between the core and the outer cover. Subsequently, the resulting billet is passed through a series of rolls to reduce it to a circular cross section. During such rolling, the change in shape of the cover and core will not be uniform, and it will be found that when the billet has been reduced to its circular form, the core will still maintain to a substantial extent its original angular shape and the corners will form projections or irregularities extending into the covering steel which will serve to key the two portions

together. In other words, the rolling operations greatly increase any natural bond between the two types of metal and this rolling is such as to create an interlock between the two. On the other hand, if one starts with a cylindrical core having an annular covering around it, and should attempt to create a bond by rolling, there is a great tendency for the cover to be actually broken away at the sides during each rolling pass, and once the bond is broken it cannot be re-stored.

When a billet has been prepared in accordance with our invention, it can be passed through a Mannesmann mill and pierced without any difficulty and without any noticeable tendency for the core and covering material to separate.

Our invention can be readily understood by reference to the accompanying drawing, in which Fig. 1 is a section of an assembly made up ready for rolling; Fig. 2 shows a sectional view of the billet prior to piercing and Fig. 3 shows a perspective view of a section of the finished product.

In the drawing, 10 is a bar of stainless steel or other high melting point corrosion resistant metal (say for example a usual type of alloy containing 18% chromium and 8% nickel) which has been electroplated with iron under conditions to avoid any intervening layer of oxide as described in said Armstrong Patent No. 1,997,538.

10 In this example the core bar 10 was surrounded by a cover of low carbon steel 14 (e. g. a steel containing .15% to .30% carbon) which is here shown as made up of two pieces which are welded together after having been shaped to receive bar 10 by machining or by the use of a dolly or by rolling. This assembly, after the usual heating, is passed through flat rolls first on one axis and then on another until all of the elements are welded into a substantially integral mass. Sub-

sequently the resulting billet is passed through a usual series of rolls to reduce it to round form, after which it usually will be turned or machined to accurate circular cross section. If a section of the resulting round product is taken, it will be found that the stainless steel core 10 has somewhat approached the circular form but still has projections as indicated at 16 where the former corners originally appeared. These corners lock the core 10 to the casing 14 as shown in Fig. 2.

50 This billet is now passed through a usual type of Mannesmann mill in which it is pierced and ordinarily enlarged in diameter (though such an enlargement is not necessary as the reduced cross sectional area of metal may if desired be made up by increased length). If a section of

the pierced tube thus formed is examined, it will be found that the corners 16 are still present and that these have been given a substantial twist so that they spiral through the tube as indicated by the dotted lines 18 in Fig. 3. Ordinarily, the corrosion resistant metal is stiffer than the low carbon steel cover and the presence of these spirally arranged projections tends to stiffen the whole tube to a greater extent than would be the case if the core were of uniform thickness. Apparently there is no appreciable tendency for the core and casing to separate.

As already stated, the core may have any desired number of sides, which means that it will have a corresponding number of projections such as those indicated at 16 in the drawings, but the projections that remain will be found to be spirally arranged as described. While we state that the core may have any desired number of sides, this statement must be given a reasonable interpretation. Naturally the number of sides must not be increased to the point where the projections of the core into the covering metal become insignificant, as it is of the very essence of our invention that the projections of the core that remain after the billet has been rolled to round form must be of sufficient magnitude to key together the metal of the core and the covering metal and thereby prevent relative movement between them under the torsional strains that result from piercing operations such as those of the Mannesmann mill.

What we claim is:

1. The method of forming composite tubes which comprises preparing a bar of a high melting point corrosion resistant metal the cross section of which forms an angled figure, enclosing such bar in a covering of corrodible steel under conditions which will permit the bar and covering to weld together, hot working the bar and cover-

ing to effect such welding, rolling and shaping the resulting billet to form a billet having a circular cross section in which the angles of the corrosion resistant bar can still be detected as irregularities of sufficient magnitude to key together the metal of the core and the covering metal and thereby prevent relative movement between them under torsional strains, and thereafter converting such billet into a tube by a rolling and piercing operation.

2. A method as specified in claim 1 in which an octagonal bar of chromium alloy steel is enclosed by welding in an assembly of low carbon steel members which are hot rolled into a substantially integral mass.

3. A method of forming composite tubes which comprises preparing a bar of high melting point corrosion resistant metal the cross section of which forms an angled figure, electroplating the surface of such bar with iron under conditions adapted to prevent the formation of a layer of oxide, enclosing such bar in a covering of corrodible steel, hot working the bar and covering to cause the two to be welded together, rolling and shaping the resulting billet to form a billet having a circular cross section in which irregularities derived from the angles of the corrosion resistant bar can still be detected, as forming projections of sufficient magnitude to key together the metal of the core and the covering metal and thereby prevent relative movement between them under torsional strains, and thereafter converting such billet into a tube by a rolling and piercing operation.

4. A method as specified in claim 3, in which the faces of the corrodible steel covering which are to be welded to the corrosion resistant bar are likewise electroplated with iron.

PERCY A. E. ARMSTRONG.  
TECUMSEH SHERMAN FITCH.